

# UNITED STATES PATENT OFFICE.

ERNST SCHULTZ, OF BERLIN, PRUSSIA, GERMANY.

## VARNISH.

SPECIFICATION forming part of Letters Patent No. 245,570, dated August 9, 1881.

Application filed March 15, 1881. (No specimens.)

*To all whom it may concern:*

Be it known that I, ERNST SCHULTZ, of Berlin, Germany, have invented a new and Improved Compound for Cleaning and Preserving Polished Wood Surfaces, of which the following is a specification.

The object of my invention is to provide a new and improved compound for removing stains from polished wood surfaces and renewing and preserving the luster of the same.

My improved compound consists of the following ingredients in the following proportions, to wit:

|    |                     |             |
|----|---------------------|-------------|
| 15 | Linseed-oil         | 350 parts   |
|    | Olive-oil           | 145 "       |
|    | Mastic              | 145 "       |
|    | Sulphuric ether     | 06 "        |
|    | Tincture of benzoin | 90 "        |
|    | Oil of turpentine   | 90 "        |
| 20 | Tincture of curcuma | 45 "        |
|    | Nitro-benzole       | 45 "        |
|    | Total               | 1,000 parts |

The linseed-oil is poured into a wooden, glass, or earthenware vessel, and the olive-oil is gradually added, the mixture being stirred continually. As soon as the two oils have become thoroughly mixed the mastic (of the best quality) is added, the mixture being stirred until it is completely dissolved. The sulphuric ether,

the tincture of benzoin, the oil of turpentine, the tincture of curcuma, and the nitro-benzole are then added in the order named, the mixture being thoroughly stirred every time a fresh ingredient is added, which ingredient is not added until the previous one has been entirely dissolved. The vessel containing the mixture is then covered, and the mixture is permitted to settle for a few hours.

The ingredients should not be mixed at a lower temperature than 70° Fahrenheit.

The mixture is applied with a brush, and is then rubbed down with a woolen cloth.

This compound is used to remove stains and congealed oil and varnish from polished wood surfaces of all kinds, and also serves to renew and preserve the polish and luster of these surfaces.

Having thus described my invention, I claim as new and desire to secure by Letters Patent—

The within-described compound for cleaning and preserving polished wood surfaces, consisting of linseed-oil, olive-oil, mastic, sulphuric ether, tincture of benzoin, oil of turpentine, tincture of curcuma, and nitro-benzole, in the proportions stated.

This specification signed by me this 4th day of February, 1881.

Witnesses: ERNST SCHULTZ,  
FRANZ SCHULTZE,  
BERTHOLD ROL.